# EUROPEAN PATENT APPLICATION

(11) **EP 4 787 404 A1**
(43) Date of publication of application: **05.08.2026**
(21) Application number: 24885852.4
(22) Date of filing: 31.10.2024
(51) Int. Cl.: H01B 13/14

(54) **METHOD FOR MANUFACTURING INSULATED WIRE, INSULATED WIRE, COIL, AND MOTOR**

(30) Priority: 31.10.2023 JP 2023187207; 04.09.2024 JP 2024152738
(71) Applicant: Mitsui Chemicals, Inc., Tokyo 104-0028 (JP)
(72) Inventor: TSUGANE, Yasuhito, Sodegaura-shi, Chiba 299-0265 (JP); WASHIO, Isao, Sodegaura-shi, Chiba 299-0265 (JP); SANO, Kouichi, Sodegaura-shi, Chiba 299-0265 (JP)
(74) Representative: Hoffmann Eitle
(86) International application number: PCT/JP2024/038973
(87) International publication number: WO 2025/095086

(57) **Abstract**

A method of producing an insulated electric wire includes: a step of pre-heating an electric conductor to a temperature that is higher than 250°C and lower than or equal to 400°C; and coating, by extrusion, the pre-heated electric conductor with a thermoplastic resin having a melting point of at least 340°C or a glass transition temperature of at least 200°C, or a resin composition containing the thermoplastic resin, thereby producing an insulated electric wire including the electric conductor and a coating film that is formed from the thermoplastic resin or the resin composition. An insulated electric wire, a coil, and a motor are also disclosed.

## Description

### Technical Field

The present disclosure relates to a method of producing an insulated electric wire, an insulated electric wire, a coil, and a motor.

### Background Art

Insulated electric wires are used in coils for industrial motors and motors for home electrical appliance. In recent years, insulated electric wires are also used in electrical motors for electric vehicles (EVs). In this field, an increased output density of a driving motor is desired from the standpoint of dynamic performance and improved fuel efficiency such as enhanced output and downsizing.

With an increase in output density, higher voltage than before is applied to insulated electric wires. Therefore, there is a possibility that insulated electric wires may experience partial electric discharge at a surface thereof, and may lead to dielectric breakdown. It is more strongly requested than before that insulated electric wires have low-dielectric properties for heat resistance and reduced partial electric discharge.

Patent Document 1 describes an insulated electric wire in which an electrically insulated film is formed on the outer circumferential surface of an electric conductor by extrusion coating with a thermoplastic polyimide.

Patent Document 1: International Publication No. 2014/084063

### SUMMARY OF INVENTION

### Problem to be Solved by Invention

As a result of earnest study conducted by the present inventors, the inventors have found that there is room for improvement in the tightness of contact between an electric conductor and a coating film in an insulated electric wire that is formed by extrusion-coating the electric conductor with an electrically insulated film containing a thermoplastic resin having a high melting point or a high glass transition point such as a thermoplastic polyimide. In a case in which the tightness of contact between the electric conductor and the coating film is low, there is a possibility that the electric insulating property of the insulated electric wire may decrease due to a gap between the electric conductor and the coating film.

A problem to be solved by one embodiment of the present disclosure is to provide a method of producing an insulated electric wire, an insulated electric wire, a coil, and a motor, in which an improved contact tightness between an electric conductor and a coating film formed from a thermoplastic resin having a melting point of at least 340°C or a glass transition temperature of at least 200°C, or a resin composition containing the thermoplastic resin is achieved, and in which the insulating property of the insulated electric wire can be improved.

### Means for Solving the Problem

Means or solving the foregoing problem include the following aspects.
<1> A method of producing an insulated electric wire, the method including:
   a step of pre-heating an electric conductor to a temperature that is higher than 250°C and lower than or equal to 400°C; and
   a step of coating, by extrusion, the pre-heated electric conductor with a thermoplastic resin having a melting point of at least 340°C or a glass transition temperature of at least 200°C, or a resin composition containing the thermoplastic resin, thereby producing an insulated electric wire including the electric conductor and a coating film that is formed from the thermoplastic resin or the resin composition.
<2> The method of producing an insulated electric wire according to <1>, wherein the thermoplastic resin is a thermoplastic resin polyimide resin.
<3> The method of producing an insulated electric wire according to <1> or <2>, wherein the electric conductor has a plated surface.
<4> The method of producing an insulated electric wire according to any one of <1> to <3>, wherein the step of coating by extrusion is a step of coating, by extrusion, the electric conductor that has been pre-heated with the thermoplastic resin or the resin composition containing the thermoplastic resin, using a pressure die.
<5> The method of producing an insulated electric wire according to any one of <1> to <4>, wherein the thermoplastic resin has a melting point of at least 340°C, and the pre-heating step is a step of pre-heating the electric conductor to a temperature that is higher than 250°C and lower than the melting point of the thermoplastic resin.
<6> The method of producing an insulated electric wire according to any one of <1> to <4>, wherein the pre-heating step is a step of pre-heating the electric conductor to a temperature that is higher than 350°C and lower than or equal to 400°C.
<7> The method of producing an insulated electric wire according to any one of <2> to <6>, wherein the thermoplastic polyimide resin includes a structural unit represented by the following Formula (1): In Formula (1), X represents a direct bond, -SO₂-, -CO-, -C(CH₃)₂-, -C(CF₃)₂-, or -S-; each of R1, R2, R3, and R4 independently represents a hydrogen atom, an alkyl group, an alkoxy group, a halogenated alkyl group, a halogenated alkoxy group, or a halogen atom; Y represents a group selected from the group consisting of the four groups respectively represented by the following Formulae (2-1) to (2-4). In the following Formulae (2-1) to (2-4), * represents a bonding position, and hydrogen atoms of aromatic rings are optionally substituted. The location of each of the bonded groups that are shown in Formula (1) without indication of the bonding positions thereof is *a para-* or *meta-* position relative to the position bound to an oxygen atom.
<8> The method of producing an insulated electric wire according to any one of <2> to <7>, wherein the thermoplastic polyimide resin includes a structural unit represented by the following Formula (3).
<9> The method of producing an insulated electric wire according to any one of <2> to <8>, wherein the thermoplastic polyimide resin includes a structural unit represented by the following Formula (6) and a structural unit represented by the following Formula (7). In Formulae (6) and (7), p/q is from 0.01 to 100.
<10> The method of producing an insulated electric wire according to any one of <2> to <9>, wherein the thermoplastic polyimide resin has a weight average molecular weight Mw of from 25,000 to 30,000.
<11> An insulated electric wire, including:
   an electric conductor; and
   a coating film that is formed from a thermoplastic resin having a melting point of at least 340°C or a glass transition temperature of at least 200°C, or a resin composition containing the thermoplastic resin,
   wherein the electric conductor and the coating film directly contact each other, and
   wherein, in a cross-section orthogonal to the longitudinal direction of the insulated electric wire, the proportion of the length of a portion at which the electric conductor and the coating film tightly contact each other to the length of the entire circumference of the electric conductor is at least 80%.
<12> The insulated electric wire according to <11>, wherein the thermoplastic resin is a thermoplastic polyimide resin.
<13> The insulated electric wire according to <11> or <12>, wherein, in a cross-section orthogonal to the longitudinal direction of the insulated electric wire, the proportion of the length of a portion at which the electric conductor and the coating film tightly contact each other to the length of the entire circumference of the electric conductor is at least 90%.
<14> The insulated electric wire according to <12> or <13>, wherein the thermoplastic polyimide resin includes a structural unit represented by the following Formula (1): In Formula (1), X represents a direct bond, -SO₂-, -CO-, -C(CH₃)₂-, -C(CF₃)₂-, or -S-; each of R1, R2, R3, and R4 independently represents a hydrogen atom, an alkyl group, an alkoxy group, a halogenated alkyl group, a halogenated alkoxy group, or a halogen atom; Y represents a group selected from the group consisting of the four groups respectively represented by the following Formulae (2-1) to (2-4). In the following Formulae (2-1) to (2-4), * represents a bonding position, and hydrogen atoms of aromatic rings are optionally substituted. The location of each of the bonded groups that are shown in Formula (1) without indication of the bonding positions thereof is *a para-* or *meta-* position relative to the position bound to an oxygen atom.
<15> A coil, including the insulated electric wire of any one of <11> to <14>.
<16> A motor, including the insulated electric wire of any one of <11> to <14>.

According to an embodiment of the present disclosure, a method of producing an insulated electric wire, an insulated electric wire, a coil, and a motor are provided in which an improved contact tightness between an electric conductor and a coating film formed from a thermoplastic resin having a melting point of at least 340°C or a glass transition temperature of at least 200°C, or a resin composition containing the thermoplastic resin is achieved, and in which the insulating property of the insulated electric wire can be improved.

### BRIEF DESCRIPTION OF DRAWINGS

Fig. 1 is a schematic structural diagram showing an example of an apparatus for use in the production method according to the present disclosure.
Fig. 2A is a schematic structural diagram showing an example of a structure of a die at an extrusion coating part of an apparatus for use in the production method according to the present disclosure.
Fig. 2B is a schematic structural diagram showing an example of a structure of a die at an extrusion coating part of an apparatus for use in the production method according to the present disclosure.

### MODES FOR CARRYING OUT THE INVENTION

Embodiments according to the present disclosure are described below. The description is provided for illustrating an embodiment, and does not limit the scope of the present disclosure. The description refers to drawings, as necessary.

In the present specification, any numerical range expressed using "to" means a range including numerical values described before and after "to" as a lower limit value and an upper limit value.

For numerical value ranges described in a stepwise manner in the present embodiment, the upper limit value or the lower limit value of one numerical value range may be replaced with the upper limit value or the lower limit value of another numerical value range in the stepwise description. The upper limit value or the lower limit value of any numerical value range described in the present embodiment may also be replaced with a value described in Examples.

In the present disclosure, the term "step" encompasses not only an independent step, but also encompasses a step that cannot be clearly distinguished from other steps, as long as the intended purpose of the step is achieved.

When an embodiment is explained with reference to a drawing in the present specification, the configuration of the embodiment is not limited to the configuration shown in the drawing. The sizes of members in each drawing are conceptual, and the relative relationship between the sizes of the members is not limited thereto.

In the present specification, each component may include plural substances that correspond to the component. In the present specification, in a case in which plural substances each corresponding to a component of interest are present in a composition, the amount of the component in the composition means the total amount of the plural substances present in the composition, unless otherwise specified.

In the present specification, the term "(meth)acrylic" may mean either of "acrylic" or "methacrylic".

### <Method of Producing Insulated Electric Wire>

An embodiment of the present disclosure is a method of producing an insulated electric wire, the method including:
pre-heating an electric conductor to a temperature that is higher than 250°C and lower than or equal to 400°C (hereinafter referred to as "pre-heating step"); and
coating, by extrusion, the pre-heated electric conductor with a thermoplastic resin having a melting point of at least 340°C or a glass transition temperature of at least 200°C (hereinafter referred to as a "highly heat-resistant thermoplastic resin") or a resin composition containing a highly heat-resistant thermoplastic resin, thereby producing an insulated electric wire including the electric conductor and a coating film that is formed from the highly heat-resistant thermoplastic resin or the resin composition containing the highly heat-resistant thermoplastic resin (hereinafter referred to as "extrusion coating step").

Due to designing the method to include the foregoing steps, contact tightness between the electric conductor and the coating film formed from the highly heat-resistant thermoplastic resin or the resin composition containing the highly heat-resistant thermoplastic resin is improved.

As described above, the insulated electric wire according to the present embodiment includes an electric conductor and a coating film that is formed from a highly heat-resistant thermoplastic resin or resin composition containing a highly heat-resistant thermoplastic resin. The coating film is provided to cover the periphery of the electric conductor and directly contact the surface of the electric conductor. The coating film serves as an electrically insulating coating for the electric conductor.

The insulated electric wire according to the present embodiment is preferably used as a wound wire for configuring a coil for a motor or the like (a magnet wire). Since the insulated electric wire according to the present embodiment has an excellent electric insulating property, the output of a motor can be increased by using the insulated electric wire according to the present embodiment as a magnet wire.

Fig. 1 is a schematic structural diagram showing an example of an apparatus for use in the method of producing an insulated electric wire according to the present disclosure. As shown in Fig. 1, an apparatus 100 includes: an unreeling part 30 for unreeling an electric conductor 20; a pre-heating part 40 for pre-heating the electric conductor 20 that has been reeled out from the unreeling part 30; an extrusion coating part 50 for extrusion-coating a highly heat-resistant thermoplastic resin or a resin composition containing a highly heat-resistant thermoplastic resin onto the pre-heated electric conductor 20 so as to form an insulated electric wire 10; a cooling part 60 for cooling the formed insulated electric wire 10; and a winding part 70 for winding-up the cooled insulated electric wire 10.

Details of the respective steps of the method of producing an insulated electric wire according to the present disclosure are described below.

### Pre-heating Step

The pre-heating step includes heating the electric conductor. The pre-heating is performed in the pre-heating part (see Fig. 1). In the pre-heating part, the electric conductor unreeled from the unreeling part is pre-heated.

### (Electric Conductor)

The electric conductor is preferably a copper wire or a wire made of a copper alloy, which has high electric conductivity, from the viewpoint of increasing the allowable electric current of the insulated electric wire. When the electric conductor is a copper wire, the copper wire is preferably made from a low-oxygen copper or an oxygen-free copper, due to excellent electric conductivity thereof. The electric conductor may be a single wire or a twisted wire.

The shape of the electric conductor preferably has a rectangular cross-sectional shape, from the viewpoint of increasing the space factor of the electric conductor in a coil formed by winding-up the insulated electric wire. In other words, the electric conductor is preferably a rectangular wire.

In regard to the wire diameter of the electric conductor, when the cross-section orthogonal to the longitudinal direction has a rectangular shape, the length of the longer side is preferably from 1.0 mm to 5.0 mm, and more preferably from 1.4 mm to 4.0 mm, for example, 2.99 mm. The length of the shorter side is preferably from 0.4 mm to 3.0 mm, and more preferably from 0.5 mm to 2.5 mm, for example, 1.54 mm. In this case, the ratio of the length of the longer side of the rectangular electric conductor to the length of the shorter side of the rectangular electric conductor (the length of the longer side of the rectangular electric conductor / the length of the shorter side of the rectangular electric conductor) is preferably from 1 to 4.

It is preferable that any paraffin used in the production of the electric conductor has been removed using an alcohol, from the viewpoint of enhancing the tightness of contact between the electric conductor and a coating film that is formed a highly heat-resistant thermoplastic resin or a resin composition containing a highly heat-resistant thermoplastic resin. It is also preferable that the electric conductor has been subjected to, for example, plating treatment so as to prevent generation of an oxide film.

The electric conductor may have been subjected to surface modification treatment, from the viewpoint of enhancing the tightness of contact between the electric conductor and a coating film that is formed a highly heat-resistant thermoplastic resin or a resin composition containing a highly heat-resistant thermoplastic resin. Examples of the surface modification treatment include: mechanical treatments such as a blast treatment, a polishing treatment, and an embossing treatment; physical treatments such as a laser treatment, a corona treatment, a plasma treatment, and a dry etching treatment; electrochemical treatments such as plating and an alumite treatment; and chemical treatments such as a chemical etching (wet etching) treatment and surface coating.

The blast treatment includes jetting particulate or fine powdery media to the electric conductor for collision, thereby providing irregularities on the surface of the electric conductor. The provision of the irregularities increases the surface roughness of the surface of the electric conductor, which facilitates anchoring of the coating film due to frictional resistance force (anchoring effect). This can improve the contact tightness between the electric conductor and the coating film. The blast treatment can also remove any oxide coating film generated on the surface of the electric conductor, and this also contributes to improvement of the contact tightness with the coating film. Therefore, blast treatment is preferable. Examples of media that can be used include those configured by metal particles, carbon particles, oxide particles, carbide particles, or nitride particles. The surface of the electric conductor may have irregularities that were imparted by processing the surface to reflect a die shape during the production of the electric conductor.

The corona treatment includes performing corona discharge treatment, thereby modifying (hydrophilizing) the surface of the electric conductor. This can result in improved contact tightness between the electric conductor and the coating film, due to chemical interactions.

The plating treatment includes coating the electric conductor with a plating material. The plating treatment is preferably wet plating, from the standpoint of costs and productivity. The plating treatment is more preferably electroless plating. Examples of the plating material include nickel plating and silver plating. The plating thickness is preferably from 0.1 to 10 µm, and more preferably from 0.5 to 5 µm.

The surface coating includes applying or spraying a coating agent onto the electric conductor, thereby performing coating. The coating can prevent surface oxidation of the electric conductor, and improves the contact tightness between the coating film and the electric conductor having the coating layer, due to chemical interactions. The coating agent to be used may be a silane coupling agent.

Examples of the silane coupling agent include vinyl trichloro silane, vinyl trimethoxy silane, vinyl triethoxy silane, 2-(3,4-epoxycyclohexyl)ethyl trimethoxy silane, 3-glycidoxypropyl trimethoxy silane, 3-glycidoxypropyl methyl diethoxy silane, 3-glycidoxypropyl triethoxy silane, p-styryl trimethoxy silane, 3-methacryloxypropyl methyl dimethoxy silane, 3-methacryloxypropyl trimethoxy silane, 3-methacryloxypropyl methyl diethoxy silane, 3-methacryloxypropyl triethoxy silane, 3-acryloxypropyl trimethoxy silane, N-2-(aminoethyl)-3-aminopropyl methyl dimethoxy silane, N-2-(aminoethyl)-3-aminopropyl trimethoxy silane, N-2-(aminoethyl)-3-aminopropyl triethoxy silane, 3-aminopropyl trimethoxy silane, 3-aminopropyl triethoxy silane, hexamethyl disilazane, 3-(2-aminoethylaminopropyl) dimethoxy methyl silane, 3-(2-aminoethylaminopropyl) trimethoxy silane, 2-(2-aminoethylthioethyl) diethoxy methyl silane, 2-(2-aminoethylthioethyl) triethoxy silane, 3-[2-(2-aminoethylaminoethylamino)propyl] trimethoxy silane, 3-triethoxysilyl-N-(1,3- dimethyl-butylidene)propylamine, N-phenyl-3-aminopropyl trimethoxy silane, N-(vinylbenzyl)-2-aminoethyl-3-aminopropyl trimethoxy silane hydrochloride, 3-ureidopropyl triethoxy silane, 3-chloropropyl trimethoxy silane, 3-isocyanatepropyl triethoxy silane, 3-mercaptopropyl methyl dimethoxy silane, 3-mercaptopropyl trimethoxy silane, bis(triethoxysilylpropyl) tetrasulfide, imidazolylalkyl-trialkoxy silane, diphenyl dimethoxy silane, hexyl trimethoxy silane, decyl trimethoxy silane, trifluoropropyl trimethoxy silane, tetramethoxy silane, tetraethoxy silane, methyl trimethoxy silane, methyl triethoxy silane, dimethyl triethoxy silane, phenyl triethoxy silane, and 3-trimethoxysilyl propyl succinic anhydride. Among these silane coupling agents, 3-aminopropyl triethoxy silane, N-2-(aminoethyl)-3-aminopropyl methyl dimethoxy silane, N-2-(aminoethyl)-3-aminopropyl trimethoxy silane, 3-aminopropyl trimethoxy silane, 3-glycidoxypropyl methyl diethoxy silane, 3-glycidoxypropyl triethoxy silane, 3-glycidoxypropyl methyl dimethoxy silane, 3-glycidoxypropyl trimethoxy silane, and the like are preferable. Commercially available silane coupling agents are also usable, and examples thereof include KBE-903, KBM-602, KBM-603, KBM903, KBE-402, KBE-403, KBM-303, KBM402, and KBM-403 (all manufactured by Shin-Etsu Chemical Co., Ltd.).

### (Pre-heating)

The pre-heating is performed such that the electric conductor becomes to have a temperature that is higher than 250°C and lower than or equal to 400°C. The pre-heating is preferably performed such that the electric conductor becomes to have a temperature that is higher than 250°C and lower than or equal to the melting point of the highly heat-resistant thermoplastic resin, and more preferably performed such that the electric conductor becomes to have a temperature that is higher than 250°C and lower than the melting point of the highly heat-resistant thermoplastic resin. Specifically, the pre-heating is preferably performed such that the electric conductor becomes to have a temperature that is higher than 250°C and lower than or equal to 388°C, and more preferably performed such that the electric conductor becomes to have a temperature that is higher than 250°C and lower than 388°C. As a result of pre-heating of the electric conductor in the foregoing temperature ranges, the temperature difference between the electric conductor and the molten highly heat-resistant thermoplastic resin or the molten resin composition containing the highly heat-resistant thermoplastic resin in the extrusion coating step will be small, as a result of which stress strain is relaxed, and, therefore, the contact tightness between the electric conductor and the coating film improves. Further, due to he temperature difference being small, the length of time during which the molten highly heat-resistant thermoplastic resin or the molten resin composition containing the highly heat-resistant thermoplastic resin, maintaining the molten state, contacts the surface of the electric conductor can be elongated. As a result, the fine irregularities formed on the surface of the electric conductor can be impregnated with the highly heat-resistant thermoplastic resin or the resin composition containing the highly heat-resistant thermoplastic resin, which leads to improved contact tightness between the electric conductor and the coating film. Further, when the pre-heating is performed such that the electric conductor becomes to have a temperature that is lower than the melting point of the highly heat-resistant thermoplastic film, an appropriately lowered flowability of the highly heat-resistant thermoplastic resin or the resin composition containing the highly heat-resistant thermoplastic resin, which is extrusion-coated on the electric conductor in the extrusion coating step, can be achieved, thereby allowing an improvement in the film thickness uniformity of the coating film while improving contact tightness.

The manner of pre-heating is not particularly limited. The pre-heating may be performed by a contact heating manner in which a heat source heated to a high temperature or flame is brought into direct contact with the electric conductor, or may be performed in a non-contact heating manner using, for example, microwaves or high-frequency waves. **In** the case of pre-heating in the non-contact heating manner, induction heating using high-frequency waves is preferable from the viewpoint of pre-heating at high temperature. The pre-heating part may be provided integrally with the unreeling part. A spool (bobbin) in the unreeling part, around which the electric conductor is wound, may be heated.

**In** a case in which the electric conductor is a copper wire and a high-frequency induction heating device is used, the pre-heating time is preferably from 0.1 seconds to 5 minutes, and more preferably from 0.1 seconds to 1 minute.

The pre-heating is performed preferably under an inert gas atmosphere such as nitrogen or argon, from the viewpoint of preventing oxidation of the surface of the electric conductor caused by high temperature and generation of an oxide film on the surface of the electric conductor.

After the pre-heating, prompt transition to the extrusion coating step is preferred so as not to lose the effect of the pre-heating step. The pre-heated electric conductor can be prevented from contacting the air, by conducting the pre-heating step and the extrusion coating step consistently in an inert gas atmosphere.

### -Extrusion Coating Step-

In the extrusion coating step, a highly heat-resistant thermoplastic resin or a resin composition containing a highly heat-resistant thermoplastic resin is extrusion-coated on the pre-heated electric conductor. The extrusion coating is performed in the extrusion coating part (see Fig. 1). In the extrusion coating part, a highly heat-resistant thermoplastic resin or a resin composition containing a highly heat-resistant thermoplastic resin, which has been melted at a predetermined temperature, is extrusion-coated on the pre-heated electric conductor fed from the pre-heating part. The thickness of the coating film is, for example, from 40 µm to 250 µm.

The resin composition is not particularly limited as far as it contains a highly heat-resistant thermoplastic resin. The resin composition may include a component, such as an additive, other than the highly heat-resistant thermoplastic resin. The resin composition may include plural highly heat-resistant thermoplastic resins.

### (Highly Heat-Resistant Thermoplastic Resin)

Examples of the thermoplastic resin having a melting point of at least 340°C or a glass transition temperature of at least 200°C (highly heat-resistant thermoplastic resin) include a thermoplastic polyimide resin and a polyether ether ketone resin (PEEK resin). The melting point of the highly heat-resistant thermoplastic resin is preferably at least 350°C, more preferably at least 360°C, still more preferably at least 370°C, and particularly preferably at least 380°C. Although the upper limit of the melting point of the highly heat-resistant thermoplastic resin is not particularly limited, the melting point is preferably at most 400°C, and more preferably at most 390°C. The glass transition temperature of the highly heat-resistant thermoplastic resin is preferably at least 210°C, more preferably at least 220°C, and still more preferably at least 230°C. Although the upper limit of the glass transition temperature of the highly heat-resistant thermoplastic resin is not particularly limited, the glass transition temperature is preferably at most 300°C, more preferably at most 290°C, still more preferably at most 280°C, and particularly preferably at most 260°C. From the viewpoint of producing an insulated electric wire, the highly heat-resistant thermoplastic resin is more preferably a thermoplastic polyimide resin. The measurement methods for the melting point and the glass transition temperature (glass transition point) are the same as those described in the Examples.

### (Thermoplastic Polyimide Resin)

Examples of the thermoplastic polyimide resin include a thermoplastic polyimide resin (a1) including a structural unit represented by the following Chemical Formula (1), a thermoplastic polyimide resin (a1)' including a structural unit represented by the following Chemical Formula (1)', a thermoplastic polyimide resin (a2) including a structural unit represented by the following Chemical Formula (3), a thermoplastic polyimide copolymer resin (a3) including a structural unit represented by the following Chemical Formula (4) and a structural unit represented by the following Chemical Formula (5), a thermoplastic polyimide resin (a4) including a structural unit represented by the following Chemical Formula (6), a thermoplastic polyimide copolymer resin (a5) including a structural unit represented by the following Chemical Formula (6) and a structural unit represented by the following Chemical Formula (7).

In Chemical Formula (1), X represents a direct bond, -SO₂-, -CO-, -C(CH₃)₂-, - C(CF₃)₂-, or -S-; each of R1, R2, R3, and R4 independently represents a hydrogen atom, an alkyl group, an alkoxy group, a halogenated alkyl group, a halogenated alkoxy group, or a halogen atom; Y represents a tetravalent aromatic group selected from the group consisting of the following connecting groups (2-1) to (2-4). The location of each of the bonded groups that are shown in Formula (1) without indication of the bonding positions thereof is *a para-* or *meta-* position relative to the position bound to an oxygen atom.

In Formula (1), the location of each of the bonded groups that are shown in Formula (1) without indication of the bonding positions thereof is preferably *meta-* position relative to the position bound to an oxygen atom. That is, Formula (1) is preferably the following Formula (1)', and the thermoplastic polyimide preferably includes a structural unit represented by the following Formula (1)'.

From the viewpoint of curbing a decrease in dielectric breakdown voltage, Y is preferably a group represented by Formula (2-1) or Formula (2-3), and more preferably a group represented by Formula (2-1).

A substituent that aromatic groups in Formulae (2-1) to (2-4) may have is preferably an alkyl group optionally having a substituent, an alkoxy group optionally having a substituent, a halogenated alkyl group optionally having a substituent, a halogenated alkoxy group optionally having a substituent, or a halogen atom. When aromatic groups in Formulae (2-1) to (2-4) have plural substituents, the substituents may be the same as or different from each other.

Here, *n in* Chemical Formulae (4) and *m in* Chemical Formula (5) represent a copolymerization ratio in the polyimide copolymer, and n/m is within a range of from 4 to 99 (mol%/mol%); n/m is more preferably from 5 to 50, still more preferably from 6 to 20, particularly preferably from 7 to 15, and most preferably 9.

Here, *p in* Chemical Formulae (6) and *q* in Chemical Formula (7) represent a copolymerization ratio in the thermoplastic polyimide copolymer, and p/q (mol%/mol%) is preferably from 0.01 to 100, more preferably from 0.1 to 50, still more preferably from 0.3 to 10, particularly preferably from 0.5 to 3, and most preferably 1.

The thermoplastic polyimide resins (a1) to (a5) presented above can be produced by providing an aromatic diamine compound and an aromatic tetracarboxylic acid dianhydride for forming the structural units shown in the corresponding chemical formula as raw materials, allowing the raw materials to react in the presence or absence of an organic solvent, and imidizing the resultant polyamide acid. Known conditions for polyimide production methods may be used for the production. At least one of the aromatic diamine compound or the aromatic tetracarboxylic acid dianhydride may be a biomass-derived compound, of which at least a part of a raw material thereof has been obtained from biomass. That is, the thermoplastic polyimide described above may be a biomass-derived thermoplastic polyimide.

The thermoplastic polyimide resin (a1)' including a structural unit represented by Chemical Formula (1)' is more specifically described as an example. An aromatic diamine compound represented by the following Chemical Formula (8) and an aromatic tetracarboxylic acid dianhydride represented by the following Chemical Formula (9) are used as raw materials.

In Chemical Formula (8), explanations for *X* and R1 to R4 are the same as the explanations for *X* and R1 to R4 in Chemical Formula (1)'.

In Chemical Formula (9), explanations for *Y* are the same as those for *Y* in Chemical Formula (1)'.

In Chemical Formulae (1), (1)', and (8), specific examples of R1, R2, R3, and R4 include a hydrogen atom, an alkyl group such as a methyl group or an ethyl group, an alkoxy group such as a methoxy group or an ethoxy group, a halogenated alkyl group such as a fluoromethyl group or a trifluoromethyl group, a halogenated alkoxy group such as a fluoromethoxy group, and a halogen atom such as a chlorine atom or a fluorine atom, among which a hydrogen atom is preferable.

In Chemical Formulae (1), (1)', and (9), *Y* is a tetravalent aromatic group selected from the group consisting of connecting groups (2-1) to (2-4) shown above, and is preferably a benzene ring. In these cases, the aromatic tetracarboxylic acid dianhydride represented by Chemical Formula (9) is pyromellitic dianhydride.

The thermoplastic polyimide resin is preferably thermoplastic polyimide resin (a1), thermoplastic polyimide resin (a1)', thermoplastic polyimide resin (a2), thermoplastic polyimide copolymer resin (a3), thermoplastic polyimide resin (a4), or thermoplastic polyimide copolymer resin (a5).

The thermoplastic polyimide preferably includes a structural unit represented by Chemical Formula (1), and more preferably consists of structural units represented by Chemical Formula (1). When the thermoplastic polyimide includes a structural unit represented by Chemical Formula (1), a coating film that is formed from the thermoplastic polyimide resin or formed from a resin composition containing the thermoplastic polyimide resin has more improved electric properties and heat resistance.

The thermoplastic polyimide more preferably includes a structural unit represented by Chemical Formula (1),' and still more preferably consists of structural units represented by Chemical Formula (1)'. When the thermoplastic polyimide includes a structural unit represented by Chemical Formula (1)', a coating film that is formed from the thermoplastic polyimide resin or formed from a resin composition containing the thermoplastic polyimide resin has more improved electric properties and heat resistance.

The thermoplastic polyimide further preferably includes a structural unit represented by Chemical Formula (3), and further more preferably consists of structural units represented by Chemical Formula (3). When the thermoplastic polyimide includes a structural unit represented by Chemical Formula (3), a coating film that is formed from the thermoplastic polyimide resin or formed from a resin composition containing the thermoplastic polyimide resin has more improved electric properties and heat resistance. When the thermoplastic polyimide includes a structural unit represented by Chemical Formula (3), the tightness of contact between the electric conductor and the coating film that is formed from the thermoplastic polyimide resin or formed from a resin composition containing the thermoplastic polyimide resin is more improved.

It is furthermore preferable that the thermoplastic polyimide further includes a structural unit represented by Chemical Formula (7), and it is particularly preferable that the thermoplastic polyimide includes a structural unit represented by Chemical Formula (1)' and a structural unit represented by Chemical Formula (7). When the thermoplastic polyimide further includes a structural unit represented by Chemical Formula (7), the tightness of contact between the electric conductor and the coating film that is formed from the thermoplastic polyimide resin or formed from a resin composition containing the thermoplastic polyimide resin is particularly improved.

In the preparation of the thermoplastic polyimide resin, one or more other aromatic diamine compounds and/or aromatic tetracarboxylic dianhydride compounds as raw materials may additionally be used for copolymerization, as far as the problem solution according to the present disclosure is not impaired.

As far as the problem solution according to the present disclosure is not impaired, plural thermoplastic polyimide resins preferred for use in the present disclosure may be freely blended, or a thermoplastic polyimide resin preferred for use in the present disclosure and another polyimide resin may be freely blended, so as to form a polymer blend.

The weight average molecular weight (Mw) of the thermoplastic polyimide is preferably greater than or equal to 20,000, from the standpoint of heat resistance. The weight average molecular weight (Mw) of the thermoplastic polyimide is preferably less than or equal to 35,000, from the standpoint of contact tightness. The weight average molecular weight (Mw) of the thermoplastic polyimide is preferably from 20,000 to 40,000, more preferably from 22,000 to 35,000, and still more preferably from 25,000 to 30,000.

In the present disclosure, the weight average molecular weight (Mw) of a thermoplastic polyimide refers to a value as measured using gel permeation chromatography (GPC). The measurement method thereof is the same as that described in the Examples. In a case in which two or more thermoplastic polyimides are used together, the value of the weight average molecular weight (Mw) thereof is a value obtained for the mixture of the two or more thermoplastic polyimides.

The melt flow rate (MFR) of the thermoplastic polyimide resin as measured at 400 °C under a load of 1.05 kg according to JIS K7210-1:2014 is not particularly limited. The MFR is preferably from 2 g/10 minutes to 30 g/10 minutes, and more preferably from 4 g/10 minutes to 20 g/10 minutes. In a case in which two or more thermoplastic polyimides are used together, the MFR thereof is a value obtained for the mixture of the two or more thermoplastic polyimides contained in the coating film. The MFR of the thermoplastic polyimide resin can be measured using a melt indexer (model number: A-371401705, manufactured by Toyo Seiki Seisaku-sho, Ltd., but the measurement instrument is not particularly limited.

The inherent viscosity of the thermoplastic polyimide resin is not particularly limited. The inherent viscosity is preferably from 0.1 dl/g to 3.0 dl/g, more preferably from 0.2 dl/g to 2.0 dl/g, still more preferably from 0.3 dl/g to 1.5dl/g, and particularly preferably from 0.4 dl/g to 1.0dl/g. When the inherent viscosity is from 0.1 dl/g to 3.0 dl/g, the molecular weight of the thermoplastic polyimide resin is within an appropriate range; as a result, a coating film formed from the thermoplastic polyimide resin or a resin composition containing the thermoplastic polyimide resin has excellent mechanical strength, and the thermoplastic polyimide resin has an excellent flowability for the preparation of a coating film formed the thermoplastic polyimide resin or a resin composition containing the thermoplastic polyimide resin by means of injection molding or extrusion molding. In a case in which two or more thermoplastic polyimides are used together, the inherent viscosity of the thermoplastic polyimide is a value obtained for the mixture of the two or more thermoplastic polyimides contained in the coating film.

The inherent viscosity is measured at a concentration of 0.5 g/100 ml in a mixed solvent of parachlorophenol/phenol (in a weight ratio of 90/10) that has been cooled to 35 °C after being heated to 200 °C. The definition of inherent viscosity is described in page 58 of "Koubunshi-Handbook" (Polymer Handbook), first edition (1995), published by Asakura Publishing Co., Ltd. and edited by The Japan Society for Analytical Chemistry.

The glass transition temperature Tg of the thermoplastic polyimide resin is not particularly limited. The glass transition temperature Tg is preferably higher than or equal to 200 °C, more preferably higher than or equal to 210 °C, still more preferably higher than or equal to 220 °C, and particularly preferably higher than or equal to 230 °C, from the standpoint of heat resistance. The glass transition temperature Tg of the thermoplastic polyimide resin is not particularly limited. The glass transition temperature Tg is preferably lower than or equal to 300 °C, more preferably lower than or equal to 290 °C, still more preferably lower than or equal to 280°C, and particularly preferably lower than or equal to 260 °C.

The glass transition temperature Tg can be obtained using a differential scanning calorimeter (model DSC220C, manufactured by Seiko Instruments Inc.); specifically, about 5 mg of the material is sealed in a measurement aluminum pan, set in the differential scanning calorimeter, heated from room temperature to 450 °C at 10 °C/minute, held at 450 °C for 5 minutes for complete melting of the resin, thereafter cooled to 30 °C at 10 °C/minute, left at 30 °C for 5 minutes, subjected to heating again to 450 °C at 10 °C/minute, and the inflection point corresponding to glass transition is taken as the glass transition temperature (Tg).

The melting point of the thermoplastic polyimide resin is not particularly limited. The melting point is preferably higher than or equal to 340 °C, more preferably higher than or equal to 350 °C, still more preferably higher than or equal to 360 °C, furthermore preferably higher than or equal to 370 °C, and particularly preferably higher than or equal to 380°C, from the standpoint of heat resistance. The melting point of the thermoplastic polyimide resin is not particularly limited. The melting point is preferably lower than or equal to 420 °C, more preferably lower than or equal to 410 °C, still more preferably lower than or equal to 400 °C, and particularly preferably lower than or equal to 390 °C, from the standpoint of mold processability.

The method used for measuring the melting point is the same as that described in the Examples.

A commercially available product of the thermoplastic polyimide resin including a repetition structural unit represented by the foregoing Formula (1') is, for example, AURUM (registered trademark; manufactured by Mitsui Chemicals, Inc. and having a glass transition temperature of 250 °C and a melting point of 388 °C).

Although the aforementioned commercially available product of the thermoplastic polyimide resin may be used, it is also possible to synthesize the thermoplastic polyimide resin using the method described below. Specifically, the thermoplastic polyimide resin can be obtained by dehydrating co-condensation of a diamine represented by the following Chemical Formula (10) and a tetracarboxylic dianhydride represented by the following Chemical Formula (11).

The method used for preparing the thermoplastic polyimide resin may include a known imidization reaction. The amount of the raw material tetracarboxylic dianhydride to be used is usually from 0.90 equivalents to 0.99 equivalents with respect to 1 equivalent of the diamine. The amount of the raw material compound to be used is preferably from 0.93 equivalents to 0.985 equivalents, and more preferably from 0.95 equivalents to 0.98 equivalents. When the amount of the raw material compound to be used is from 0.90 equivalents to 0.99 equivalents, the molecular weight of the thermoplastic polyimide resin is sufficiently high, as a result of which a coating film formed from the thermoplastic polyimide resin or from a resin composition containing the thermoplastic polyimide resin would have excellent mechanical properties, and the thermoplastic polyimide resin would have excellent flowability.

The synthesis of the thermoplastic polyimide resin preferably includes blocking the reaction terminals of molecules, for example, with phthalic anhydride. Blocking of the reaction terminals remarkably improves the thermal stability of the thermoplastic polyimide resin.

The reaction is particularly preferably performed in an organic solvent. Examples of the organic solvent include N,N-dimethylformamide, N,N-diethylacetamide, N,N-dimethoxyacetamide, N-methyl-2-pyrrolidone, 1,3-dimethyl-2-imidazolidinone, N-methylcaprolactam, 1,2-dimethoxyethane, bis(2-methoxyethyl) ether, 1,2-bis(2-methoxyethoxy)ethane, bis[2-(2-methoxyethoxy)ethyl] ether, tetrahydrofuran, 1,3-dioxane, 1,4-dioxane, pyrroline, picoline, dimethylsulfoxide, dimethylsulfone, tetramethylurea hexamethylphosphoramide, phenol, o-cresol, m-cresol, p-cresol, p-chlorophenol, anisole, benzene, toluene, and xylene. The organic solvent may be used singly or in mixture of two or more thereof.

The reaction temperature is usually from room temperature to 250 °C, and preferably from 140 °C to 200 °C. The reaction pressure is not particularly limited, and sufficient reaction can be performed at normal pressure. The reaction time varies with the solvent and the reaction temperature, and the reaction time is usually from 4 to 24 hours. In regard to imidization methods, a desired polyimide resin can be obtained by heating a polyamide acid as a precursor to a temperature of from 100 °C to 300 °C for imidization, or by performing chemical imidization using an imidization agent such as acetic anhydride.

As far as the properties of the highly heat-resistant thermoplastic resin are not impaired, additives may include at least one selected from the group consisting of carbon fiber, glass fiber, potassium titanate fiber, aluminum borate fiber, metal fiber, ceramic fiber, boron fiber, silicon carbide fiber, asbestos fiber, rock wool fiber, and aramid fiber.

As far as the properties of the highly heat-resistant thermoplastic resin are not impaired, additives may include at least one of a filler, a sliding agent, a release agent, a stabilizer, a coloring agent, a crystal nucleating agent, or the like, if necessary, such as mica, synthetic mica, wollastonite, talc, silicone oil, fluorine-containing oil, glass beads, molybdenum disulfide, clay, silica, alumina, diatomite, earth, hydrated alumina, Shirasu Balloon, carbon nanotube, calcium carbonate, hydrotalcite, fluorine, or graphite (for example, artificial graphite, natural graphite (for example, vein graphite, flake graphite, amorphous graphite) , or the like).

As far as the properties of the highly heat-resistant thermoplastic resin are not impaired, additives may include, if necessary, at least one selected from the group consisting of various liquid crystal polymers, thermoplastic resins that are different from the highly heat-resistant thermoplastic resin (for example, fluororesins, polyether imide, polyether nitrile, polyether ketone, polyether ketone ketone, polyether ketone ether ketone ketone, polyamide imide, polyether sulfone, polysulfone, polyarylate, and/or polyphenylene sulfide), and thermosetting resins (for example, epoxy resins, polybenzimidazole resins, and polyimide resins).

In a case in which the resin composition includes an additive, the content of the additive and the content of the highly heat-resistant thermoplastic resin are not particularly limited, and may be selected, as appropriate, depending on the additive type and the like. The content of the additive is preferably within the following ranges.

The content of the additive is preferably from 0% by mass to 40% by mass with respect to the total amount of the resin composition. The content of the highly heat-resistant thermoplastic resin is preferably from 60% by mass to 100% by mass with respect to the total amount of the resin composition.

The highly heat-resistant thermoplastic resin or the resin composition containing the highly heat-resistant thermoplastic resin is preferably in a pellet state.

### (Extrusion Coating)

Extrusion coating is performed using an extruder. Examples of the extruder include a single-screw extruder, a twin screw extruder, and an L-type extruder.

An extruder includes: a hopper configured to supply a highly heat-resistant thermoplastic resin or a resin composition containing a highly heat-resistant thermoplastic resin; a screw configured to melt-knead the highly heat-resistant thermoplastic resin or the resin composition containing a highly heat-resistant thermoplastic resin; a cylinder configured to extrude the highly heat-resistant thermoplastic resin or the resin composition containing a highly heat-resistant thermoplastic resin; and a die configured to mold the highly heat-resistant thermoplastic resin or the resin composition containing a highly heat-resistant thermoplastic resin so as to produce an insulated electric wire, and the extruder further includes a heating device configured to heat the cylinder, and a filter configured to remove contaminants.

The hopper is preferably purged with an inert gas such as nitrogen or argon or vacuumed, from the viewpoint of reducing the generation of carbides on the screw or the cylinder. However, this treatment is not essential.

The design of the screw is not particularly limited. The design may be selected, as appropriate, from a full flight design, a rapid compression design, a gradual compression design, a barrier flight design, a mixing flight design, or the like.

The effective length L of the screw is, for example, 625 mm.

The screw diameter D is, for example, Φ25 mm.

The ratio (L/D) of the screw effective length L to the screw diameter D is, for example, 25.

The compression ratio of the screw (the ratio between the flight groove depths of cylinder portions C-1 and C-3) is, for example, 3.0.

The number of revolutions of the screw is, for example, 3.0 rpm.

The heating temperature of the extruder is, for example from 390 °C to 400 °C at a cylinder portion C-1, for example from 410 °C to 420 °C at a cylinder portion C-2, for example from 420 °C to 430 °C at a cylinder portion C-3, for example from 420 °C to 430 °C at a neck portion, for example from 420 °C to 430 °C at a head portion, and for example from 410 °C to 420 °C at a die portion.

The die is preferably a cross-head die. The die diameter is, for example, Φ7.2 mm. The die tip may have a diameter of Φ6.0 mm and a length of 9.0 mm.

Preferable die structures include a die structure having a sleeve provided around an electric conductor as illustrated in Fig. 2A, and a pressure die structure as illustrated in Fig. 2B. With respect to the die structure, the pressure die structure illustrated in Fig. 2B is more preferable than the die structure having a sleeve provided around an electric conductor illustrated in Fig. 2A. The die illustrated in Fig. 2B includes an electric conductor feed path through which an electric conductor is fed, and an extrusion channel for a resin, and further includes a contact path 22 which extends from the extrusion part tip (extrusion port) Q of the die toward the upstream in the extrusion direction, and in which the resin contacts the circumferential face of the electric conductor. Since the die structure is the pressure die structure illustrated in Fig. 2B, the molten resin is brought into contact with the electric conductor in a state in which the static pressure of the molten resin is increased by compression at the internal clearance, thereby enhancing the contact tightness between the electric conductor and the coating film.

The die land length if preferably longer, from the viewpoint of allowing the molten highly heat-resistant thermoplastic resin or the molten resin composition containing the highly heat-resistant thermoplastic resin to flow well and enhancing the tightness of contact between the electric conductor and the coating film by means of an increased back pressure.

The filter mesh is preferably less than 200 mesh from the viewpoint of decreasing the resin pressure, and is, for example, from 30 mesh to 100 mesh. Plural types of mesh may be combined.

The feed velocity of the electric conductor to the extruder may be from 1 mm/minute to 300 mm/minute.

Extrusion coating may be performed with an increased degree of vacuum in the cylinder. Increasing the degree of vacuum lowers the tendency toward generation of an oxide layer on the surface of the electric conductor, which leads to an enhanced affinity between the electric conductor and the coating film and enhanced contact tightness.

According to the method according to one embodiment of the present disclosure described above, an insulated electric wire is produced. In the insulated electric wire, the contact tightness between the electric conductor and the coating film is enhanced. The produced insulated electric wire is wound around a winding part (see Fig. 1), but the following steps may also be included.

The method according to the present disclosure may further include a step of cooling the coated electric conductor (i.e., the insulated electric wire) (hereinafter also referred to as "cooling step"), in addition to the aforementioned steps.

In the cooling step, the insulated electric wire is cooled. The cooling is performed in a cooling part (see Fig. 1). The cooling may be air-cooling or water-cooling.

The method according to the present disclosure may further include a step of holding at a temperature that is in a range of from [the heating temperature at the extrusion coating part (for example, the die portion) -10°C] to [the heating temperature at the extrusion coating part +10°C] (hereinafter also referred to as a "temperature holding step"), after the extrusion coating step but before the cooling step. Inclusion of the temperature holding step improves the affinity between the electric conductor and the coating film, thereby improving the contact tightness between the electric conductor and the coating film.

The method according to the present disclosure may further include a post-heating step, after the extrusion coating step but before the cooling step. This further heating performed after the extrusion coating improves the affinity between the electric conductor and the coating film, thereby improving the contact tightness between the electric conductor and the coating film.

The method according to the present disclosure may further include a rolling step, after the extrusion coating step but before the cooling step. Rolling the produced insulated electric wire at a predetermined pressure improves the contact tightness between the electric conductor and the coating film. The rolling can be performed using, for example, a roll press, a cold isotactic press (CIP), or the like.

The aforementioned various conditions for the respective steps of the method of producing an insulated electric wire may be combined, as appropriate. For example, a process may be carried out in which a Ni-plated rectangular copper wire is used as an electric conductor, the process including degreasing the copper wire with alcohol, thereafter pre-heating this electric conductor to a temperature range of from 300 °C to 400 °C by means of high-frequency induction heating, and performing extrusion coating using a pressure die as a die. In the pre-heating, the atmosphere surrounding the electric conductor may be an inert gas atmosphere.

### <Insulated Electric Wire>

The insulated electric wire according to the present disclosure is an insulated electric wire that includes an electric conductor, and a coating film formed from a highly heat-resistant thermoplastic resin or a resin composition containing a highly heat-resistant thermoplastic resin,
the electric conductor and the coating film directly contacting each other, and
in a cross-section orthogonal to the longitudinal direction of the insulated electric wire, the proportion of the length of the portion at which the electric conductor and the coating film tightly contact each other (hereinafter also simply referred to as "tight contact portion") to the length of the entire circumference of the electric conductor being at least 80%. **In** other words, the proportion of the length of a portion at which a gap is present between the electric conductor and the coating film to the length of the entire circumference of the electric conductor in a cross-section orthogonal to the longitudinal direction of the insulated electric wire is at least 20%.

Configuring the insulated electric wire such that the proportion of the length of the tight contact portion to the length of the entire circumference is at least 80% in a cross-section orthogonal to a longitudinal direction of the insulated electric wire enhances the tightness of contact between the electric conductor and the coating film, thereby curbing deterioration of the electrically insulating property of the insulated electric wire. The proportion of the length of the tight contact portion to the length of the entire circumference in a cross-section orthogonal to a longitudinal direction of the insulated electric wire can be measured using the method described in the Examples.

From the viewpoint of contact tightness between the electric conductor and the coating film, the proportion of the length of the tight contact portion to the length of the entire circumference of the electric conductor in a cross-section orthogonal to a longitudinal direction of the insulated electric wire is preferably at least 90%, more preferably at least 95%, still more preferably at least 97%, and particularly preferably at least 98%.

The specifics of the electric conductor and the specifics of the highly heat-resistant thermoplastic resin or a resin composition containing the highly heat-resistant thermoplastic resin are as described in the explanation of the method of producing an insulated electric wire.

In the insulated electric wire according to the present disclosure, the highly heat-resistant thermoplastic resin is preferably a thermoplastic polyimide resin, and the thermoplastic polyimide resin preferably includes a structural unit represented by the following Formula (1).

In Formula (1), X represents a direct bond, -SO₂-, -CO-, -C(CH₃)₂-, -C(CF₃)₂-, or -S-; each of R1, R2, R3, and R4 independently represents a hydrogen atom, an alkyl group, an alkoxy group, a halogenated alkyl group, a halogenated alkoxy group, or a halogen atom; Y represents a group selected from the group consisting of four groups respectively represented by the following Formulae (2-1) to (2-4) wherein, in the following Formulae (2-1) to (2-4), * represents a bonding position, and hydrogen atoms of aromatic rings are optionally substituted; and the location of each of bonded groups that are shown in Formula (1) without indication of bonding positions thereof is *a para-* or *meta-* position relative to the position bound to an oxygen atom.

The insulated electric wire according to the present disclosure can be produced according to the aforementioned method of producing an insulated electric wire.

### <Coil>

The use of the insulated electric wire according to the present disclosure is not particularly limited. Since the insulated electric wire according to the present disclosure has high contact tightness between the electric conductor and the coating film and has excellent electrically insulating properties, the insulated electric wire can suitably be used in coils such as coils of motors. A coil can be obtained by winding up an insulated electric wire in a coil shape. The insulated electric wire according to the present disclosure can be formed into a coil by being wound in a coil shape.

### <Motor>

The insulated electric wire according to the present application can be, after being formed into a coil, combined with a stator so as to configure a motor. In this case, the coil is preferably in a state of being wound around a rotor, from the viewpoint of preparing a motor.

### EXAMPLES

One embodiment of the present disclosure is more specifically described below by reference to examples. This embodiment of the present disclosure is not limited to the examples described below.

### -Preparation-

The following materials were prepared.
- Electric Conductor (Copper Wire):
   Round wire A (having a diameter of 2 mm; not Ni-plated)
   Round wire B (having a diameter of 2 mm; Ni-plated (from 2 to 3 µm))
   Rectangular wire C (having a thickness of 1.54 mm and a width of 2.99 mm, with a curvature radius of corners of 6 mm; not Ni-plated)
   Rectangular wire D (having a thickness of 1.54 mm and a width of 2.99 mm, with a curvature radius of corners of 6 mm; Ni-plated (from 2 to 3 µm))
- Highly heat-resistant thermoplastic resin or a resin composition containing a highly heat-resistant thermoplastic resin:
   TPI1 to TPI5

TPI1 to TPI5 were synthesized according to the following procedures.

### (Synthesis Example 1)

Thermoplastic polyimide resin TPI1 (with a medium molecular weight) that contains a structural unit represented by Formula (3) was synthesized according to the following procedures.

A container equipped with a stirrer, a reflux condenser, a water separator, and a nitrogen introduction tube was placed. 2.886 kg (7.8 mol) of 4,4'-bis(3-aminophenoxy)biphenyl, 1.604 kg (7.37 mol) of pyromellitic dianhydride, 0.148 kg (1.0 mol) of phthalic anhydride, and 21.53 kg of m-cresol were charged into the container. Then, the temperature was increased to 200 °C with stirring in a nitrogen atmosphere, during which removal of about 350 mol of water by distillation was confirmed. Then, the reaction was allowed to proceed at 200 °C for 6 hours. Thereafter, cooling to room temperature was performed, and 10.8 kg of toluene was added thereto. Thereafter, filtration was performed to obtain yellow polyimide powder. This polyimide powder was washed with toluene, and then dried at 180 °C for 24 hours, thereby obtaining 5.46 kg (yield: 98.5%) of polyimide powder (thermoplastic polyimide). This polyimide powder was extruded at 400 °C using a Takayasu Φ25 mm extruder, and a pellet was obtained. This thermoplastic polyimide resin TPI1 was found to have a melting point of 388 °C, a glass transition temperature of 245 °C, and an imide group density of 25.5%. The melting point and glass transition temperature of the thermoplastic polyimide resin were measured using a differential scanning calorimeter (DSC) (model DSC220C manufactured by Seiko Instruments Inc.) (the same applies to the respective synthesis examples provided below). Thermoplastic polyimide resin TPI1 was found to have a weight average molecular weight (Mw) of 32,500.

The weight average molecular weight Mw of thermoplastic polyimide resin TPI1 was measured using gel permeation chromatography (GPC) as follows. The weight average molecular weights Mw of other thermoplastic polyimide resins in the Examples were measured in the same manner. 1.5 mL of 4-chlorophenol was added to 5 mg of the sample, and gently stirred at from 130 °C to 140 °C. After the resultant solution was air-cooled to room temperature, 3.5 mL of chloroform was added. Thereafter, filtration was performed using a 0.2 µm filter, so as to prepare a sample solution. Measurement was carried out under the following conditions, using the prepared sample solution.
Detection device: differential refraction index meter RI (RI-8020 manufactured by Tosoh Corporation)
Columns: two columns of TSK gel GMHXL and one column of G2500 HXL (manufactured by Tosoh Corporation, having an internal diameter of 7.8 mm and a length of 300 mm)
Column temperature: 23 °C
Solvent: 4-chlorophenol/chloroform (3/7) (volume/volume)
Flow rate: 0.8 mL/min
Sample Concentration: 1 mg/mL
Injection volume: 0.3 mL
Standard samples: Monodisperse polystyrenes manufactured by Tosoh Corporation

### (Synthesis Example 2)

Thermoplastic polyimide resin TPI2 (with a low molecular weight) that contains a structural unit represented by Formula (3) was synthesized according to the following procedures.

A container equipped with a stirrer, a reflux condenser, a water separator, and a nitrogen introduction tube was placed. 2.886 kg (7.8 mol) of 4,4'-bis(3-aminophenoxy)biphenyl, 1.582 kg (7.25 mol) of pyromellitic dianhydride, 0.148 kg (1.0 mol) of phthalic anhydride, and 21.53 kg of m-cresol were charged into the container. Then, the temperature was increased to 200 °C with stirring in a nitrogen atmosphere, during which removal of about 350 mol of water by distillation was confirmed. Then, the reaction was allowed to proceed at 200 °C for 6 hours. Thereafter, cooling to room temperature was performed, and 10.8 kg of toluene was added thereto. Thereafter, filtration was performed to obtain yellow polyimide powder. This polyimide powder was washed with toluene, and then dried at 180 °C for 24 hours, thereby obtaining 5.46 kg (yield: 98.5%) of polyimide powder (powder of a thermoplastic polyimide). This polyimide powder was extruded at 400 °C using a Takayasu Φ25 mm extruder, and a pellet was obtained. This thermoplastic polyimide resin TPI2 was found to have a melting point of 386 °C, a glass transition temperature of 240 °C, and an imide group density of 25.5%. Thermoplastic polyimide resin TPI2 was found to have a weight average molecular weight (Mw) of 28,200. The Mw value was measured by the above-described method.

### (Synthesis Example 3)

Thermoplastic polyimide resin TPI3 (with a high molecular weight) that contains a structural unit represented by Formula (3) was synthesized according to the following procedures.

A container equipped with a stirrer, a reflux condenser, a water separator, and a nitrogen introduction tube was placed. 2.873 kg (7.8 mol) of 4,4'-bis(3-aminophenoxy)biphenyl, 1.570 kg (7.46 mol) of pyromellitic dianhydride, 0.148 kg (1.0 mol) of phthalic anhydride, and 21.53 kg of m-cresol were charged into the container. Then, the temperature was increased to 200 °C with stirring in a nitrogen atmosphere, during which removal of about 350 mol of water by distillation was confirmed. Then, the reaction was allowed to proceed at 200 °C for 6 hours. Thereafter, cooling to room temperature was performed, and 10.8 kg of toluene was added thereto. Thereafter, filtration was performed to obtain yellow polyimide powder. This polyimide powder was washed with toluene, and then dried at 180 °C for 24 hours, thereby obtaining 5.46 kg (yield: 98.5%) of polyimide powder (powder of a thermoplastic polyimide). This polyimide powder was extruded at 400 °C using a Takayasu Φ25 mm extruder, and a pellet was obtained. This thermoplastic polyimide resin TPI3 was found to have a melting point of 389 °C, a glass transition temperature of 248 °C, and an imide group density of 25.5%. Thermoplastic polyimide resin TPI3 was found to have a weight average molecular weight (Mw) of 36,900. The Mw value was measured by the above-described method.

### (Synthesis Example 4)

Thermoplastic polyimide resin TPI4 that contains a structural unit represented by Formula (4) and a structural unit represented by Formula (5) was synthesized according to the following procedures.

A container equipped with a stirrer, a reflux condenser, a water separator, and a nitrogen introduction tube was placed. 3.312 kg (9.0 mol) of 4,4'-bis(3-aminophenoxy)biphenyl, 0.2 kg (1.0 mol) of 4,4'-diaminodiphenyl ether, 2.071 kg (9.5 mol) of pyromellitic dianhydride, 0.148 kg (1.0 mol) of phthalic anhydride, and 21.53 kg of cresol acid were charged into the container. Then, the temperature was increased to 145 °C with stirring in a nitrogen atmosphere, during which removal of about 350 mol of water by distillation was confirmed. Then, the reaction was allowed to proceed at 145 °C for 4 hours. Thereafter, cooling to room temperature was performed, and 10.8 kg of methyl ethyl ketone was added thereto. Thereafter, filtration was performed to obtain yellow polyimide powder. This polyimide powder was washed with methyl ethyl ketone, and then dried at 180 °C for 24 hours, thereby obtaining 5.26 kg (yield: 98%) of polyimide powder (thermoplastic polyimide). This polyimide powder was extruded at 400 °C using a Takayasu Φ25 mm extruder, and a pellet was obtained. This thermoplastic polyimide resin TPI4 was found to have a glass transition temperature of 253 °C and an imide group density of 23.9%, but the melting point of thermoplastic polyimide resin TPI4 could not be determined. In thermoplastic polyimide resin TPI4, the ratio of structural units represented by Formula (4) to structural units represented by Formula (5) was 9:1.

### (Synthesis Example 5)

Thermoplastic polyimide resin TPI5 that contains a structural unit represented by Formula (6) and a structural unit represented by Formula (7) was synthesized according to the following procedures.

A container equipped with a stirrer, a reflux condenser, a water separator, and a nitrogen introduction tube was placed. 3.684 kg (10.0 mol) of 4,4'-bis(3-aminophenoxy)biphenyl, 1.081 kg (4.96 mol) of pyromellitic dianhydride, 1.459 (4.86 mol) of 3,3',4,4'-biphenyl tetracarboxylic dianhydride, 0.148 kg (1.0 mol) of phthalic anhydride, and 21.53 kg of m-cresol were charged into the container. Then, the temperature was increased to 200 °C with stirring in a nitrogen atmosphere, during which removal of about 350 mol of water by distillation was confirmed. Then, the reaction was allowed to proceed at 200 °C for 6 hours. Thereafter, cooling to room temperature was performed, and 10.8 kg of methanol was added thereto. Thereafter, filtration was performed to obtain yellow polyimide powder. This polyimide powder was washed with methanol, and then dried at 180 °C for 24 hours, thereby obtaining 5.46 kg (yield: 98.5%) of polyimide powder (powder of a thermoplastic polyimide). This polyimide powder was extruded at 400 °C using a Takayasu Φ25 mm extruder, and a pellet was obtained. This thermoplastic polyimide resin TPI5 was found to have a glass transition temperature of 235 °C and an imide group density of 23.9%, but the melting point of thermoplastic polyimide resin TPI5 could not be determined. In thermoplastic polyimide resin TPI5, the ratio of structural units represented by Formula (6) to structural units represented by Formula (7) was 1:1.

### <Example 1>

An extruder equipped with a die (screw: full flight with a diameter of 20 mm, L/D=24, compression ratio: 3.0) was placed. The heating temperature in the cylinder portion of the extruder was controlled with respect to three divided zones, which were named C1, C2, and C3 in the order from the material charge side. The heating temperature was set to 380 °C for C1 zone, 410 °C for C2 zone and C3 zone, and 420 °C for the head portion located downstream the cylinder of the extruder and the die located at the tip of the head portion. The shape of the opening of the die was geometrically similar to the cross-sectional shape of the electric conductor.

A conductive wire (round wire A) as an electric conductor was heated to 260 °C (pre-heating step). The pellet of thermoplastic polyimide resin TPI1 was charged into the extruder, and molten resin of the TPI1 pellet was directly coated on the outer circumferential face of the electric conductor (copper wire, round wire A) pre-heated at 260 °C (extrusion coating step), and allowed to cool. As a result, an insulated electric wire of Example 1 was obtained.

The insulated electric wire included the electric conductor and a coating film that directly covers the electric conductor. The coating film was formed of thermoplastic polyimide resin TPI1. The outer shape of the cross-section of the insulated electric wire was geometrically similar to the shape of the electric conductor. The thickness of the coating film was 120 µm.

The pre-heating was performed with a preheater, and the temperature of the pre-heated copper wire was measured just before the cross-head. The measurement of the pre-heating temperature was performed using a moving wire thermometer (MW-33ETC1ASP .manufactured by Anritsu Meter Co. Ltd.).

### -Contact Tightness Test-

A straight-line-shaped test piece having a length of about 300 mm was stretched for 15% at a rate of 5±1 mm per second using a tensile tester (product name: AUTOGRAPH AGS-J, manufactured by Shimadzu Corporation), according to the Contact Tightness Test specified in JIS C 3216-3 5.5. A cut that reached the electric conductor was made in the coating film along one revolution at nearly the center of the test piece, and, after stretching, the occurrence of peeling or detachment of the coating film was checked in one test piece wire. In a case in which detachment of the coating film was observed, the length of the portion at which the coating film detached, starting from the cut position, was measured. All of the four faces of the test piece were checked, and the maximum peeling distance was evaluated. The evaluation was conducted according to the following criteria. The results are shown in Table 1.
A: The maximum peeling distance was from 0 mm to 5 mm.
B: The maximum peeling distance was from more than 5 mm to 10 mm.
C: The maximum peeling distance was more than 10 mm.

**In** the evaluation, rank B is a lowest target level that should be satisfied, and rank A is a particularly superior level for a product.

### <Examples 2 to 34 and Comparative Examples 1 to 13>

An electric conductor was extrusion coated, and the contact tightness between the electric conductor and a coating film was evaluated, in the same manner as that in Example 1, except that the electric conductor (copper wire), the coating material (a highly heat-resistant thermoplastic resin or a resin composition containing a highly heat-resistant thermoplastic resin), the pre-heating temperature for the electric conductor, the die structure, and the like were replaced by those shown in Tables 1 to 9. The results are shown in Tables 1 to 9.

**Table 1**

| | Comparative Example 1 | Comparative Example 2 | Example 1 | Example 2 | Example 3 |
|---|---|---|---|---|---|
| Electric Conductor (Copper Wire) | Round Wire A | Round Wire A | Round Wire A | Round Wire A | Round Wire A |
| Coating Material | TPI1 | TPI1 | TPI1 | TPI1 | TPI1 |
| Coating Thickness (µm) | 120 | 120 | 120 | 120 | 120 |
| Die Type | Die A | Die A | Die A | Die A | Die A |
| Electric Conductor Pre-heating Temperature | 150 | 200 | 260 | 300 | 350 |
| Contact Tightness | C | C | B | B | A |
| Peeling Distance (mm) | 35 | 35 | 10 | 8 | 5 |

| | | | | | |
|---|---|---|---|---|---|
| Die A: Tubing Die, Die B: Pressure Die | | | | | |

**Table 2**

| | Comparative Example 3 | Comparative Example 4 | Example 4 | Example 5 | Example 6 |
|---|---|---|---|---|---|
| Electric Conductor (Copper Wire) | Round Wire A | Round Wire A | Round Wire A | Round Wire A | Round Wire A |
| Coating Material | TPI1 | TPI1 | TPI1 | TPI1 | TPI1 |
| Coating Thickness (µm) | 120 | 120 | 120 | 120 | 120 |
| Die Type | Die B | Die B | Die B | Die B | Die B |
| Electric Conductor Pre-heating Temperature | 150 | 200 | 260 | 300 | 350 |
| Contact Tightness | C | C | B | B | A |
| Peeling Distance (mm) | 35 | 35 | 9 | 6 | 4 |

| | | | | | |
|---|---|---|---|---|---|
| Die A: Tubing Die, Die B: Pressure Die | | | | | |

**Table 3**

| | Comp. Ex. 5 | Comp. Ex. 6 | Ex. 7 | Ex. 8 | Ex. 9 | Ex. 10 | Ex. 11 |
|---|---|---|---|---|---|---|---|
| Electric Conductor (Copper Wire) | Round Wire B | Round Wire B | Round Wire B | Round Wire B | Round Wire B | Round Wire B | Round Wire B |
| Coating Material | TPI1 | TPI1 | TPI1 | TPI1 | TPI1 | TPI1 | TPI1 |
| Coating Thickness (µm) | 120 | 120 | 120 | 120 | 120 | 80 | 240 |
| Die Type | Die A | Die A | Die A | Die A | Die A | Die A | Die A |
| Electric Conductor Pre-heating Temperature | 150 | 200 | 260 | 300 | 350 | 350 | 350 |
| Contact Tightness | C | C | B | A | A | A | A |
| Peeling Distance (mm) | 35 | 35 | 7 | 3 | 0.1 | 0.1 | 0.1 |

| | | | | | | | |
|---|---|---|---|---|---|---|---|
| Die A: Tubing Die, Die B: Pressure Die, Ex.: Example, Comp. Ex.: Comparative Example | | | | | | | |

**Table 4**

| | Comp. Ex. 7 | Comp. Ex. 8 | Ex. 12 | Ex. 13 | Ex. 14 | Ex. 15 | Ex. 16 |
|---|---|---|---|---|---|---|---|
| Electric Conductor (Copper Wire) | Round Wire B | Round Wire B | Round Wire B | Round Wire B | Round Wire B | Round Wire B | Round Wire B |
| Coating Material | TPI1 | TPI1 | TPI1 | TPI1 | TPI1 | TPI1 | TPI1 |
| Coating Thickness (µm) | 120 | 120 | 120 | 120 | 120 | 80 | 240 |
| Die Type | Die B | Die B | Die B | Die B | Die B | Die B | Die B |
| Electric Conductor Pre-heating Temperature | 150 | 200 | 260 | 300 | 350 | 350 | 350 |
| Contact Tightness | C | C | A | A | A | A | A |
| Peeling Distance (mm) | 35 | 35 | 5 | 2 | 0.05 | 0.05 | 0.05 |

| | | | | | | | |
|---|---|---|---|---|---|---|---|
| Die A: Tubing Die, Die B: Pressure Die, Ex.: Example, Comp. Ex.: Comparative Example | | | | | | | |

**Table 5**

| | Comparative Example 9 | Comparative Example 10 | Example 17 | Example 18 | Example 19 |
|---|---|---|---|---|---|
| Electric Conductor (Copper Wire) | Rectangular Wire C | Rectangular Wire C | Rectangular Wire C | Rectangular Wire C | Rectangular Wire C |
| Coating Material | TPI1 | TPI1 | TPI1 | TPI1 | TPI1 |
| Coating Thickness (µm) | 120 | 120 | 120 | 120 | 120 |
| Die Type | Die A | Die A | Die A | Die A | Die A |
| Electric Conductor Pre-heating Temperature | 150 | 200 | 260 | 300 | 350 |
| Contact Tightness | C | C | B | B | A |
| Peeling Distance (mm) | 35 | 35 | 10 | 8 | 5 |

| | | | | | |
|---|---|---|---|---|---|
| Die A: Tubing Die, Die B: Pressure Die, | | | | | |

**Table 6**

| | Comparative Example 11 | Example 20 | Example 21 | Example 22 | Example 23 |
|---|---|---|---|---|---|
| Electric Conductor (Copper Wire) | Rectangular Wire C | Rectangular Wire C | Rectangular Wire C | Rectangular Wire C | Rectangular Wire C |
| Coating Material | TPI1 | TPI1 | TPI1 | TPI1 | TPI1 |
| Coating Thickness (µm) | 100 | 100 | 100 | 100 | 100 |
| Die Type | Die B | Die B | Die B | Die B | Die B |
| Electric Conductor Pre-heating Temperature | 200 | 260 | 300 | 350 | 380 |
| Contact Tightness | C | B | B | A | A |
| Peeling Distance (mm) | 35 | 9 | 6 | 4 | 4 |

| | | | | | |
|---|---|---|---|---|---|
| Die A: Tubing Die, Die B: Pressure Die, | | | | | |

**Table 7**

| | Comparative Example 12 | Example 24 | Example 25 | Example 26 |
|---|---|---|---|---|
| Electric Conductor (Copper Wire) | Rectangular Wire D | Rectangular Wire D | Rectangular Wire D | Rectangular Wire D |
| Coating Material | TPI1 | TPI1 | TPI1 | TPI1 |
| Coating Thickness (µm) | 120 | 120 | 120 | 120 |
| Die Type | Die A | Die A | Die A | Die A |
| Electric Conductor Pre-heating Temperature | 200 | 260 | 300 | 360 |
| Contact Tightness | C | B | A | A |
| Peeling Distance (mm) | 35 | 7 | 3 | 0.1 |

| | | | | |
|---|---|---|---|---|
| Die A: Tubing Die, Die B: Pressure Die, | | | | |

**Table 8**

| | Comparative Example 13 | Example 27 | Example 28 | Example 29 | Example 30 |
|---|---|---|---|---|---|
| Electric Conductor (Copper Wire) | Rectangular Wire D | Rectangular Wire D | Rectangular Wire D | Rectangular Wire D | Rectangular Wire D |
| Coating Material | TPI1 | TPI1 | TPI1 | TPI1 | TPI1 |
| Coating Thickness (µm) | 120 | 120 | 120 | 120 | 120 |
| Die Type | Die B | Die B | Die B | Die B | Die B |
| Electric Conductor Pre-heating Temperature | 200 | 260 | 300 | 350 | 380 |
| Contact Tightness | C | A | A | A | A |
| Peeling Distance (mm) | 35 | 5 | 2 | 0.05 | 0.05 |

| | | | | | |
|---|---|---|---|---|---|
| Die A: Tubing Die, Die B: Pressure Die, | | | | | |

**Table 9**

| | Example 30 | Example 31 | Example 32 | Example 33 | Example 34 |
|---|---|---|---|---|---|
| Electric Conductor (Copper Wire) | Rectangular Wire D | Rectangular Wire D | Rectangular Wire D | Rectangular Wire D | Rectangular Wire D |
| Coating Material | TPI1 | TPI2 | TPI3 | TPI4 | TPI5 |
| Coating Thickness (µm) | 120 | 120 | 120 | 120 | 120 |
| Die Type | Die B | Die B | Die B | Die B | Die B |
| Electric Conductor Pre-heating Temperature | 380 | 380 | 380 | 380 | 380 |
| Contact Tightness | A | A | A | A | A |
| Peeling Distance (mm) | 0.05 | 0.03 | 0.06 | 0.05 | 0.02 |

| | | | | | |
|---|---|---|---|---|---|
| Die A: Tubing Die, Die B: Pressure Die, | | | | | |

Based on the results shown in Table 1, it is seen that pre-heating of the electric conductor to a temperature that is higher than 250 °C but lower than or equal to 400 °C resulted in a small peeling distance and improved contact tightness between the electric conductor and the coating film compared to a case in which the temperature is outside the foregoing range (Examples 1 to 3 vs. Comparative Examples 1 and 2). A higher pre-heating temperature for the electric conductor resulted in a greater improvement of the contact tightness (Examples 1 to 3).

As shown in Table 2 (and Table 1), adopting a pressure die as the die structure resulted in a even smaller peeling distance and more improved contact tightness (Example 1 vs. Example 4, Example 2 vs. Example 5, Example 3 vs. Example 6).

As shown in Table 3 (and Table 1), use of a plated electric conductor resulted in a drastically smaller peeling distance and drastically improved contact tightness, as compared to a case with no plating. In particular, in cases in which the electric conductor was heated at a pre-heating temperature of 350 °C, the peeling distance was drastically smaller and improvement of contact tightness was conspicuous (Example 3 vs. Example 9). No difference due to coating thickness was found (Examples 9 to 11).

As shown in Table 4 (and Table 3), replacement of the die structure with a pressure die resulted in a smaller peeling distance and more improved contact tightness (Example 7 vs. Example 12, Example 8 vs. Example 13, Example 9 vs. Example 14, Example 10 vs. Example 15, and Example 11 vs. Example 16). Here, comparison between a case with plating and a case without plating revealed that the plating brought about a drastically smaller peeling length and a drastically improved contact tightness (Example 6 vs. Example 14; see Table 4 and Table 2).

Even when the shape of the electric conductor (copper wire) was varied as indicated in Table 5, contact tightness between the electric conductor and the coating film improved upon pre-heating of the electric conductor to a temperature that is higher than 250 °C and lower than or equal to 400 °C. A higher pre-heating temperature for the electric conductor resulted in a more improved contact tightness (Examples 17 to 19).

Also in this case, replacement of the die structure with a pressure die resulted in an even smaller peeling distance and further improved contact tightness (Example 19 vs. Example 22), as shown in Table 6 (and Table 5). Contact tightness in a case in which the pre-heating temperature for the electric conductor was 350 °C and contact tightness in a case in which the pre-heating temperature for the electric conductor was 380 °C were at a comparable level.

Provision of plating to the electric conductor resulted in a drastically smaller peeling distance and a drastically improved contact tightness (Example 26 vs. Example 19), as shown in Table 7 (and Table 5).

Further, as shown in Table 8 (and Table 7), replacement of the die structure with a pressure die resulted in a still smaller peeling distance and further improved contact tightness (Example 26 vs. Example 29). In this case, comparison between a case with plating and a case without plating revealed that the plating brought about a drastically smaller peeling length and a drastically improved contact tightness (Example 22 vs. Example 29, and Example 23 vs. Example 30; see Table 8 and Table 6). Contact tightness in a case in which the pre-heating temperature for the electric conductor was 350 °C and contact tightness in a case in which the pre-heating temperature for the electric conductor was 380 °C were at a comparable level (Example 29 vs. Example 30). These two cases exhibited superior contact tightness compared to a case in which the pre-heating temperature for the electric conductor was a lower temperature.

As shown in Table 9, studies in which the coating material was varied under a condition in which the pre-heating temperature for the electric conductor was 380 °C, in which the die structure was a pressure die, and in which plating was performed, TPI5, which includes a structural unit represented by Formula (6) and a structural unit represented by Formula (7), exhibited the best contact tightness (Example 34), and TPI2 (with low molecular weight), which includes a structural unit represented by Formula (3), exhibited the second best contact tightness (Example 31).

With respect to Examples 29 and 30 and Comparative Examples 12 and 13, the proportion of the length of the tight contact portion to the length of the entire circumference of the electric conductor in a cross-section of the insulated electric wire was also determined.

### -Proportion of Length of Tight Contact Portion to Length of Entire Circumference in Cross-Section-

The proportion of the length of a portion at which the electric conductor and the coating film tightly contacted (tight contact portion) to the length of the entire circumference of the electric conductor was determined according to the following procedures.

The respective insulated electric wires prepared in Examples 29 and 30 and Comparative Examples 12 and 13 were cut in a cross-section that was orthogonal to the longitudinal direction of the insulated electric wire, embedded in an epoxy resin, and the cross-section was exposed by mechanical polishing. Then, the cross-section was observed at a 500-fold magnifications using a microscope (VHX-X1) manufactured by Keyence Corporation, and a micrograph was obtained. The obtained micrograph was image-analyzed by using image-processing software, and length L1 of the entire circumference of the electric conductor, length L2 of a portion at which a gap was present between the electric conductor and the coating film, and length L3 of a portion (tight contact portion) at which the electric conductor and the coating film tightly contact with no gap present between the electric conductor and the coating film were respectively determined. From the determination results, the proportion of the length of the tight contact portion to the length of the entire circumference of the electric conductor was calculated (L3/L1×100). The determination, and the calculation of the proportion were performed for three cross-sections of each insulated electric wire, and the average value thereof was taken as the proportion of the length of the tight contact portion to the length of the entire circumference. The results are shown in Table 10.

**Table 10**

| | Comparative Example 12 | Comparative Example 13 | Example 29 | Example 30 |
|---|---|---|---|---|
| Electric Conductor (Copper Wire) | Rectangular Wire D | Rectangular Wire D | Rectangular Wire D | Rectangular Wire D |
| Coating Material | TPI1 | TPI1 | TPI1 | TPI1 |
| Coating Thickness (µm) | 120 | 120 | 120 | 120 |
| Die Type | Die A | Die B | Die B | Die B |
| Electric Conductor Pre-heating Temperature | 200 | 200 | 350 | 380 |
| Contact Tightness | C | C | A | A |
| Peeling Distance (mm) | 35 | 35 | 0.05 | 0.05 |
| Proportion of Tight Contact Portion in Cross-Section (%) | 18.6 | 40.0 | 98.7 | 99.0 |

| | | | | |
|---|---|---|---|---|
| Die A: Tubing Die, Die B: Pressure Die, | | | | |

As shown in Table 10, it is seen that insulated electric wires obtained after pre-heating the electric conductor to a temperature that is higher than 250°C and lower than or equal to 400°C have excellent contact tightness between the electric conductor and the coating film, which is demonstrated not only by the peeling distances but also by the results in which the proportion of the length of the tight contact portion to the length of the entire circumference of the electric conductor was higher than or equal to 98% in cross-sections of the insulated electric wires.

The disclosure of Japanese Patent Application No. 2023-187207, filed October 31, 2023, and the disclosure of Japanese Patent Application No. 2024-152738, filed September 4, 2024, are incorporated herein by reference in their entirety.

All publications, patent applications, and technical standards mentioned in this specification are herein incorporated by reference to the same extent as if each individual publication, patent application, or technical standard was specifically and individually indicated to be incorporated by reference.

### Explanation of Reference Characters

100: Apparatus for Producing Insulated electric wire
10: Insulated Electric Wire
20: Electric Conductor
22: Contact Path
30: Unreeling Part
40: Pre-heating Part
50: Extrusion Coating Part
60: Cooling Part
70: Winding Part
200: Die (Cross-head Die)
Q: Tip of Extrusion Part (Extrusion Port)
R: Resin

## Claims

1. A method of producing an insulated electric wire, the method comprising:
a step of pre-heating an electric conductor to a temperature that is higher than 250°C and lower than or equal to 400°C; and
a step of coating, by extrusion, the pre-heated electric conductor with a thermoplastic resin having a melting point of at least 340°C or a glass transition temperature of at least 200°C, or a resin composition containing the thermoplastic resin, thereby producing an insulated electric wire including the electric conductor and a coating film that is formed from the thermoplastic resin or the resin composition.

2. The method of producing an insulated electric wire according to claim 1, wherein the thermoplastic resin is a thermoplastic resin polyimide resin.

3. The method of producing an insulated electric wire according to claim 1, wherein the electric conductor has a plated surface.

4. The method of producing an insulated electric wire according to claim 1, wherein the step of coating by extrusion is a step of coating, by extrusion, the electric conductor that has been pre-heated with the thermoplastic resin or the resin composition containing the thermoplastic resin, using a pressure die.

5. The method of producing an insulated electric wire according to claim 1, wherein the thermoplastic resin has a melting point of at least 340°C, and the pre-heating step is a step of pre-heating the electric conductor to a temperature that is higher than 250°C and lower than the melting point of the thermoplastic resin.

6. The method of producing an insulated electric wire according to claim 1, wherein the pre-heating step is a step of pre-heating the electric conductor to a temperature that is higher than 350°C and lower than or equal to 400°C.

7. The method of producing an insulated electric wire according to claim 2, wherein the thermoplastic polyimide resin includes a structural unit represented by the following Formula (1): wherein, in Formula (1), X represents a direct bond, -SO₂-, -CO-, -C(CH₃)₂-, - C(CF₃)₂-, or -S-; each of R1, R2, R3, and R4 independently represents a hydrogen atom, an alkyl group, an alkoxy group, a halogenated alkyl group, a halogenated alkoxy group, or a halogen atom; Y represents a group selected from the group consisting of four groups respectively represented by the following Formulae (2-1) to (2-4) wherein, in the following Formulae (2-1) to (2-4), * represents a bonding position, and hydrogen atoms of aromatic rings are optionally substituted; and a location of each of bonded groups that are shown in Formula (1) without indication of bonding positions thereof is *a para-* or *meta-* position relative to a position bound to an oxygen atom:

8. The method of producing an insulated electric wire according to claim 7, wherein the thermoplastic polyimide resin includes a structural unit represented by the following Formula (3):

9. The method of producing an insulated electric wire according to claim 7, wherein the thermoplastic polyimide resin includes a structural unit represented by the following Formula (6) and a structural unit represented by the following Formula (7): wherein, in Formulae (6) and (7), p/q is from 0.01 to 100.

10. The method of producing an insulated electric wire according to claim 7, wherein the thermoplastic polyimide resin has a weight average molecular weight Mw of from 25,000 to 30,000.

11. An insulated electric wire, comprising:
an electric conductor; and
a coating film that is formed from a thermoplastic resin having a melting point of at least 340°C or a glass transition temperature of at least 200°C, or a resin composition containing the thermoplastic resin,
wherein the electric conductor and the coating film directly contact each other, and
wherein, in a cross-section orthogonal to a longitudinal direction of the insulated electric wire, a proportion of a length of a portion at which the electric conductor and the coating film tightly contact each other to a length of an entire circumference of the electric conductor is at least 80%.

12. The insulated electric wire according to claim 11, wherein the thermoplastic resin is a thermoplastic polyimide resin.

13. The insulated electric wire according to claim 11, wherein, in a cross-section orthogonal to a longitudinal direction of the insulated electric wire, a proportion of a length of a portion at which the electric conductor and the coating film tightly contact each other to a length of an entire circumference of the electric conductor is at least 90%.

14. The insulated electric wire according to claim 12, wherein the thermoplastic polyimide resin includes a structural unit represented by the following Formula (1): wherein, in Formula (1), X represents a direct bond, -SOz-, -CO-, -C(CH₃)₂-, - C(CF₃)₂-, or -S-; each of R1, R2, R3, and R4 independently represents a hydrogen atom, an alkyl group, an alkoxy group, a halogenated alkyl group, a halogenated alkoxy group, or a halogen atom; Y represents a group selected from the group consisting of four groups respectively represented by the following Formulae (2-1) to (2-4) wherein, in the following Formulae (2-1) to (2-4), * represents a bonding position, and hydrogen atoms of aromatic rings are optionally substituted; and a location of each of bonded groups that are shown in Formula (1) without indication of bonding positions thereof is *a para-* or *meta-* position relative to a position bound to an oxygen atom:

15. A coil, comprising the insulated electric wire of any one of claims 11 to 14.

16. A motor, comprising the insulated electric wire of any one of claims 11 to 14.
